

# UNITED STATES PATENT OFFICE.

FRANK M. TAYLOR, OF SIOUX CITY, IOWA, ASSIGNOR TO THOMAS C. BRENNAN, OF NEWCASTLE, NEBRASKA, AND MAURICE W. BRENNAN, OF WYNOT, NEBRASKA.

## POLISHING COMPOSITION.

1,410,041.

Specification of Letters Patent. Patented Mar. 21, 1922.

No Drawing.

Application filed April 9, 1921. Serial No. 459,989.

To all whom it may concern:

Be it known that I, FRANK M. TAYLOR, a citizen of the United States, and a resident of Sioux City, in the county of Woodbury 5 and State of Iowa, have invented certain new and useful Improvements in Polishing Compositions, of which the following is a specification.

This invention has for its object the production of an improved polishing composition particularly adapted for polishing varnished surfaces, and so compounded as to give a high lustre to the surface, yet leaving no grease thereon.

15 Furthermore the invention contemplates a polishing composition adapted to give a high lustre to varnished surfaces, which may be applied with a minimum of effort and which will not injure nor deaden the original lustre of a highly polished varnish surface.

My composition consists of the following ingredients combined preferably in the proportions stated:

|                                              | Per cent. |
|----------------------------------------------|-----------|
| 25 5 oz. denatured alcohol                   | 31.25     |
| 10 oz. paraffin oil                          | 62.5      |
| $\frac{1}{2}$ oz. shellac (preferably white) | 3.125     |
| $\frac{1}{3}$ oz. oil of citronella          | .7812     |
| $\frac{1}{4}$ oz. alkanet root               | 1.5625    |
| 30 $\frac{1}{8}$ oz. oil of mirbane          | .7812     |

The above ingredients are intimately mixed and applied to the surface preferably with a soft rag and then rubbed dry with a soft, dry rag.

Having thus described the invention, what I claim is:—

1. A surface polishing composition comprising denatured alcohol, paraffin oil, shellac, oil of citronella, alkanet root and oil of mirbane.

2. A polishing composition consisting of the following ingredients combined approximately in the per cents stated, to wit: 40 5 oz. denatured alcohol, 31.25%, paraffin oil, 62.5%, shellac (preferably white), 45 3.125%, oil of citronella, .7812%, alkanet root, 1.5625%, oil of mirbane, .7812%.

In testimony whereof I have hereunto set my hand this 16th day of March, 1921.

FRANK M. TAYLOR.